

# UNITED STATES PATENT OFFICE.

AUGUST LENDLE, OF FOREST HILLS, NEW YORK, ASSIGNOR TO KUTTROFF PICKHARDT & CO., INC., OF NEW YORK, N. Y., A CORPORATION OF NEW YORK.

## METHOD OF PRECIPITATING ACID COLORS.

1,378,418.

Specification of Letters Patent. Patented May 17, 1921.

No Drawing.

Application filed September 9, 1920. Serial No. 409,246.

*To all whom it may concern:*

Be it known that I, AUGUST LENDLE, a citizen of the United States, residing at Forest Hills, county of Queens, and State 5 of New York, have invented new and useful Improvements in Methods of Precipitating Acid Colors, of which the following is a specification.

My invention comprises a new and improved method of precipitating certain acid colors. It is well known that many acid colors (such as scarlet, orange, alkali-blue, etc.,) are precipitated with salts, such as, for instance, chlorid of barium, chlorid of 15 calcium, sugar of lead, etc.

Heretofore, it has not been feasible to precipitate other acid colors (such as patent blue, acid green, erioglaucin, soluble blue, acid violet, etc.,) with the same precipitating agents.

I have discovered that acid dyestuffs such as patent blue, acid green, erioglaucin, soluble blue, acid violet, etc., can now be precipitated substantially completely and perfectly if any of the known precipitating agents such as chlorid of barium, sugar of lead, etc., are used in connection with complex acids or their salts, containing an acid (such as phosphoric or silicic and tungsten 25 or molybdenum.

The object of the present invention is to precipitate these colors into insoluble or difficultly soluble coloring matters in the presence or absence of substrata (such as, 35 hydrate of alumina, blanc fixe, etc.). These then obtained coloring matters, or "lakes" are suitable for the manufacture of paints, printing inks, lithographic inks, etc.

The following is an example of suitable

procedure, but the invention is not restricted to this example.

100 lbs. acid green are dissolved in water to make a 1% solution; to this is added a 10% watery solution of 200 lbs. chlorid of barium and then a 10% watery solution of 45 sodium phospho tungstate.

In the above process molybdenum is the equivalent of tungsten and the salts of complex acids are the equivalents of said acids. In the claims, therefore, the word "tungsten" 50 will be read to include molybdenum and the word "acid" will be read to include its salts.

I claim:

1. The method of precipitating acid colors, which consists in treating the same with a 55 precipitating agent, and a complex acid containing an acid and tungsten.

2. The method of precipitating acid colors, which consists in treating the same with a precipitating agent, and a complex acid containing phosphorus and tungsten. 60

3. A coloring matter lake containing the combination of an acid coal tar coloring matter with a precipitating agent, and a complex acid containing an acid and tungsten. 65

4. A coloring matter lake containing the combination of an acid coal tar coloring matter with a precipitating agent, and a complex acid containing phosphorus and tungsten. 70

In testimony whereof I have hereunto set my hand in the presence of two subscribing witnesses.

AUGUST LENDLE.

Witnesses:

W.M. P. PICKHARDT,  
H. STOLZE.